# EUROPEAN PATENT SPECIFICATION

(11) **EP 0 441 879 B1**
(45) Date of publication and mention of the grant of the patent: **15.07.1998**
(21) Application number: 89912908.4
(22) Date of filing: 07.11.1989
(51) Int. Cl.: B65D 23/08

(54) **GLASS CONTAINER COATING PROCESS**
VERFAHREN ZUR BESCHICHTUNG AUF EINEM GLASBEHÄLTER
PROCEDE D'APPLICATION D'UN REVETEMENT SUR UN RECIPIENT EN VERRE

(30) Priority: 07.11.1988 US 267877
(43) Date of publication of application: 21.08.1991
(73) Proprietor: BRANDT MANUFACTURING SYSTEMS, INC., Deposit, NY 13754 (US)
(72) Inventor: BRANDT, Thomas, L., Windsor, NY 13865 (US); WILLKENS, Daniel, N., Elmira, NY 14905 (US)
(74) Representative: Jenkins, Peter David
(86) International application number: US8904886
(87) International publication number: WO9005667

(56) References cited:
- GB-A- 2 021 124
- US-A- 3 083 854
- US-A- 3 859 117
- US-A- 3 937 853
- US-A- 4 053 076
- US-A- 4 268 554
- US-A- 4 860 906
- WORLD PATENTS INDEX LATEST Week 8644, Derwent Publications Ltd., London, GB; AN 86-287859 & JP-A-61 209 927 (FUJIKURA KASEI K.K.) 18 September 1986
- WORLD PATENTS INDEX LATEST Week 8520, Derwent Publications Ltd., London, GB; AN 85-119959 & JP-A-60 060 947 (YAMAMURA GLASS) 8 April 1985
- PATENT ABSTRACTS OF JAPAN vol. 12, no. 382 (C-535)(3229) 12 October 1988 & JP-A-63 129 038 ( KOA GLASS ) 1 June 1988
- PATENT ABSTRACTS OF JAPAN vol. 11, no. 8 (C-396)(2455) 9 January 1987 & JP-A-61 186 249 ( POLA CHEM. IND. INC. ) 19 August 1986

## Description

The invention relates to a method of coating glass containers, and more particularly to a technique for applying colour coatings that singularly or together may be coloured, block ultra-violet light, and offer a range of surface textures.

The glass container industry limits itself to three primary colours for containers; clear glass (commonly called flint glass), amber and green. The green and amber are melted in several hues for both product differentiation and protection of the contents from the adverse effects of transmitted visual light as well as the ultra-violet component of natural and artificial light. Significant cost resulting from lost production when a glass melting unit changes from one colour to another is experienced throughout the industry as well as the cost to carry inventory of containers made of a specific color during a run of a few weeks that will satisfy many months of need. There is also an ongoing cost of glass raw materials necessary for coloring, as well as the additional cost of storage silos and batch material weighing apparatus. In addition, extra fuel is required to melt colored glass batch. Also, the melting furnace life is reduced by the corrosive action of colored glass batches.

Recycling of glass containers has become a very popular and cost effective way to deal with empty glass container disposal. One problem of the existing system is the need to segregate the various colors of glass so as not to contaminate the different glass melts. This segregation requires three separate systems from the empty container receiving station throughout all of the handling up to and including the charging of the melting unit with the proper color glass. Introduction of expensive machinery is required to separate containers collected without segregation.

It is common practice in the glass industry to treat the outer surface of the containers with materials to counteract the effects of high glass-to-glass friction experienced on freshly manufactured glass products. Glass containers are conveyed with a great deal of glass-to-glass contact and at times considerable line pressure. Without treatment there is considerable visible scratching which may result in breakage. It is common to surface treat at two (2) locations in the operation. Immediately after forming and before lehring, the containers pass through a vapor which leaves a tin oxide film bonded to the surface. After lehring, the containers are sprayed with a dilute water solution of a material which, after evaporation of the water, leaves a film to provide surface lubricity. Of the two treatments, the tin oxide film is most costly, both for materials and system maintenance. The lubricity of the second film, though needed to prevent surface damage, may cause problems in subsequent labeling of the container.

There is an ongoing program in the container industry to reduce the weight of the container by reducing wall thickness, but still maintain acceptable product strength for both the internal pressures of carbonated beverages and the impact strength to survive handling damage in the filling operations, in the market place and by the consumer. The benefits of reduced weight are economic: lower glass melting fuel and material costs, higher container manufacturing speeds (lower cost) and reduced product shipping costs.

Patent Abstracts of Japan, Vol. 12, No. 382 (C-535) (3229) discloses the painting of a bottle surface for shielding ultra-violet rays following a method according to the preambles of claims 1 and 13. World Patent Index Latest, Week 8644, Derwent Publications Ltd., London, GB, AN 86-28759 discloses a UV shielding covering composition for glass.

It is an aim of the present invention, with certain variations, to overcome the above described glass industry problems and limitations.

More particularly, it is an aim of this invention to provide a technique for colouring glass containers which is economic, environmentally sound and offers product protection not heretofore available.

It is a further aim of this invention to provide a method for applying the materials to glass containers in line with the container manufacturing process, i.e., 500 containers per minute.

It is a further aim to provide a colour coated glass container with improved impact resistance and abrasion resistance.

It is a still further aim of the invention to eliminate the need for a tin oxide coating.

Yet another aim of this invention is to foster continued further reduction in container weight.

The present invention provides a method of coating a glass container, comprising the steps of: providing a container of glass, said glass having an inside surface directed toward an interior of said container and an outer surface directed toward an exterior of said container; annealing said glass container; coating said container with at least a final acrylic coating layer applied in liquid form; and curing said acrylic coating; said method being characterized by the steps of applying a first coating material to said container at a first location in a container fabrication line subsequent to said annealing step; conveying said container to a second location with said first coating material providing surface lubricity; and applying an acrylic coating layer which is compatible with said first coating material over said glass on said outer surface of said container while at least some of said first coating material remains on said outer surface, said acrylic coating layer having a cured thickness of no greater than 0.0152 mm (0.0006 inch).

The present invention further provides a method of coating a glass container, comprising the steps of: providing a container of glass, said glass having an inside surface directed toward an interior of said container and an outer surface directed toward an exterior of said container; annealing said glass container; coating said glass container with at least a final acrylic coating layer applied in liquid form; and curing said acrylic coating; said method being characterized by the steps of applying a first coating material to said container at a first location in a container fabrication line subsequent to said annealing step; conveying said container to a second location with said first coating material providing surface lubricity; exposing said first coating material to an oxidizing flame whereby first coating material is burnt off; and applying an acrylic coating layer over said glass on said outer surface of said container subsequent to said oxidizing flame step, said acrylic coating layer having a cured thickness of no greater than 0.0152 mm (0.0006 inch).

Thus, the aims and advantages of the invention are achieved by coating the glass containers with a material, preferably heat-curable or UV-curable acrylic, which provides impact resistance and durability, such that it is no longer necessary to provide the tin oxide film prior to container lehring. The coating material is selected to have a colour corresponding to the desired container colour, and/or can be selected to have a composition which will block certain wavelengths of light which are considered harmful to the contents of the bottle. The coating material also provides sufficient impact and abrasion resistance to permit the tin oxide film to be dispensed with, with merely a token amount of the lubricating film being applied after annealing. This lubricating film is one which is compatible with the coating, such as ammonium stearate. The lubicating flim is sufficient to enable damage-free conveying from the lehr, through the inspection stations and into the colour coat machine staging area.

It has been demonstrated that a container coated with a nominal 0.0152 mm (0.6 mil) of the coating will survive a 30-40% increase in fracture impact over an uncoated container.

An embodiment of the present invention will now be described hereinbelow, with reference to the accompanying drawing, which illustrates a bottle processing system for practicing the present invention.

The present invention resides in applying to a clear glass container a coating which may have a number of properties. There are a great number of properties which may be considered significant in any given case, but the properties discussed herein are color, light blocking for protection of the container contents from irradiation, abrasion resistance and impact resistance. The coating material is preferably a urethane coating, with appropriate additives as will be described below.

The first significant property of the coating material is the color. As described above, it is sometimes desirable to color the bottle, e.g., to amber or green, and this has heretofore been achieved by specific formulation of the glass batch introduced into the melters. Through the use of suitable additives, an acrylic coating (e.g., urethane), either heat-curable or UV-curable, could be made to provide the desired coloring of the container. The coloring technique would provide any color desired to suit the particular product, from light tints to fully opaque colors. The particular additives to be used for this purpose would depend on the colors desired, with a number of suitable organic dyes being well-known to those of skill in the art.

By coloring the glass after melting, many benefits are possible. To change from one color class to another it is now necessary to completely drain a melting unit, flush and refill with the new color. In other cases, it may be possible to change by adding colored batch to clear, but even this results in a period of unusable glass until the output is uniformly colored. In any case, there is lost production time, usually a week, or more. According to the present invention, this lost time would be eliminated since only the clear glass would be required. The availability of any colored glass on demand would be of great interest to the container users. A major savings in batch material required for coloring glass would also be obtained.

Because the coating would burn off completely in the melting unit at the high furnace temperatures, the recycling of glass containers would be greatly facilitated. The present need to segregate glass containers by colors would be eliminated if all containers were clear glass and colored after manufacture. This would be of particular benefit to the collecting stations and recycling facilities responsible for the glass recycling programs.

The cured color coat is formulated to withstand the wash and pasteurization processes associated with non-returnable containers, and with chemical modifications to the color coat, returnable containers will be able to survive the alkali wash required prior to refilling. Nor will the color coat be adversely affected by water, alcohol or organic materials used in the filling operations.

The color coatings on adjacent containers will not abrade each other during the filling and packaging operations associated with transport, store display and consumer purchasing, and the color coat will also be chemically and physically stable.

It is known that it is necessary to protect some container contents, e.g., beer, from adverse effects in flavor (known as "sunstruck taste" in the brewing industry) due to prolonged exposure to natural and artificial light. This protection may in part be offered by amber glass, commonly used as a beer container, although neither green glass or clear (flint) glass offer protection. Further, even the protection afforded by amber glass decreases as the bottle becomes thinner. According to the present invention, suitable light blocking agents can be added to the topcoat to protect the container contents. By coating the outside surface uniformly, complete protection is achieved irrespective of container wall thickness.

A preferred technique for providing irradiation protection for the container contents is to determine, e.g., via spectrographic analysis, which wavelengths of light are absorbed by the container contents, and to then include additives in the topcoat which will block light in these regions. Again, the additives to be used would be known to those of skill in the art after determining the wavelengths of light to be blocked. The damaging ultra-violet component may be largely blocked by a clear additive, either to a clear or colored coating.

It has been demonstrated by this invention, that protection can be secured by the addition of various selected colorants and UV blocking agents to the coating material.

Variations in color coating texture and appearance may also be desirable. It has been demonstrated that with changes in coating composition the surface may be altered from gloss finish, to matte, to frosted. This is done without sacrificing physical properties.

In addition to providing desired container coloring and content irradiation protection, a further aim of the invention to eliminate the cost of tin oxide coating. Because the acrylic coating of this invention provides impact resistance and durability, it is no longer necessary to provide the tin oxide film prior to container lehring. A lubricating film is sufficient to enable damage-free conveying from the lehr, through the inspection stations and into the color coat machine staging area. It should be a lubricating film compatible with the coating, such as ammonium stearate. Alternatively, it could be a film which may be easily burned off prior to the coating process, although in the preferred embodiment the ammonium stearate is comaptible with the coating material and allows the bonding of the coating to the glass so that burning off of residual lubricant may not be necessary. For some container applications, however, it may be desirable to remove the stearate coating prior to coating.

As described above, it is yet another aim of this invention to foster continued further reduction in container weight. It has been demonstrated that a container coated with a nominal 0.0152 mm (0.6 mil) of the coating will survive a 30-40% increase in fracture impact over an uncoated container. In addition, the light blockage is no longer affected by the thickness of the glass, so that glass thickness is only limited by strength considerations.

It is also well known that considerable glass surface damage occurs throughout the container handling cycle including bulk and case packing at the container manufacturer. At the container filling operations, the handling surface damage is severe also. Because the coating provides a much greater degree of surface protection, container failure from surface damage would be greatly reduced. The applied layer of coating is complete over the entire surface without voids, or discontinuities. Further reductions in wall thickness without compromising container strength are therefore possible. These reductions have value in increasing container manufacturing speeds, reducing fuel usage and material costs as well as reducing transportation costs.

It may also be advantageous to use a coupling agent to promote adhesion of the color coat material to the container surface to meet certain container processing and use requirements, specifically, but not limited to the typical beer industry pasteurization process. While the coupling agent can be mixed with the color coat before application, it may be desirable to apply the coupling agent to the container surface before the color coat is applied for economic reasons as well as technical reasons.

It has been demonstrated that all three materials, i.e., the ultraviolet block, colorant, and coupling agent can be applied together in one solution and at one spray operation.

To receive the coating, the containers are conveyed into a multi-station spray system which has been designed to address the needs of uniform coverage of the container and recovery of the overspray.

In the event the materials are sprayed, it is desirable to prevent any material from contacting the finish of the container. This is the area including the opening, top seal surface, thread or closure cover area and protuberance immediately below. This could be accomplished using a container gripper device designed to completely cover the area described above, e.g., with a split housing which, when closed, dovetails to form a barrier to the spray material. Dipping and flow coating are other processes that may be used to apply the coating.

The gripper devices are attached to a conveyor network whose design allows for spacing of the glass containers to optimize the coating and curing of the coating materials. The grippers should also be designed for rotating the container at the spraying and curing positions to insure uniform coating and processing.

Rather than spraying, the application of the coating solution could be accomplished by belt or roller coating as described in WO-A-90/05088. Alternative methods of applying the topcoat include, but are not limited to, the use of a roller shaped to conform to the contour of the container, a belt flexible enough to conform to the container contour, or flowing the coating over the container while it is slowly rotated. Dipping may also be advantageous. Each option has its own merits and must be weighed against economics, quality and production rates.

The containers are then conveyed to a circulating hot air cure chamber designed to provide the necessary exposure to hot air to completely cure the topcoat. It has been demonstrated that air moving at 457.2 m (1500 feet) per minute and at a temperature of 287.8°C (550°F) will insure a complete cure in 1.5 minutes.

Immediately following cure of the topcoat, the container can be packaged for shipment and subsequent wash, filling and pasteurization, if required, by the various food and beverage packaging operations.

The single figure herein illustrates one example of a system for applying the coating of this invention. The coating with ammonium stearate would be performed before the bottles are received at the upper right of the figure along a conveyor 100. The bottles would then be transferred to a loading station 104 one at a time by a star wheel control device 102. The bottles are then moved downwardly onto an indexing table 106 by means of a suitable placement device. The indexing table 106 will include container holders, e.g., suction holders or the like, and there may be supports at the neck of each container to absorb pressure during the container transfer.

After loading three bottles onto the indexing table 106, the indexing table is then rotated counterclockwise from the loading station to a container orienting station generally designated at reference character 108. If desired or necessary for the particular type of container being used, the container may here be rotated to a particular orientation, although this will be unnecessary in many container systems. The rotating of the container would preferably be performed by rotation of individual container holder suction cups on the indexing table 106 until the correct position is detected, e.g., by suitable photo-electric means, at which point the holders would be locked in their correct positions.

If it is desirable to burn off residual lubricant, this can be done at station 108, in addition to proper orienting of the bottles, preferably by an oxidizing flame but alternatively by other means such as corona treatment.

After proper orienting of the bottles and optional removal of lubricant, the indexing table 106 is further rotated to bring the bottles to the coating station 114 where the coating of this invention is applied.

The indexing table 106 is then further rotated to bring the coated bottles to an unloading station where each container is off-loaded onto a container conveyor. There are a number of ways in which the bottles could be removed. All bottles could be removed from the indexing table 106 to a single conveyor 120, taking care to ensure that the coatings are not disturbed. It may, be necessary, with suitable care taken, to use an air knife. It may, however, be necessary to move the bottles by clamping them at their "finish" and carrying them onto the conveyor 120 in a known manner.

It is also to be remembered that the bottles are held in groups of three on the indexing table 106. In the interest of speed, it would be possible to arrange three separate conveyors 120 each for receiving one of the three bottles in each group from the indexing table 106.

Once on the conveyor 120, the coating on the bottles is cured in a suitable manner, e.g., by heat in the case of heat-curable coating or by U-V energy in the case of UV-curable coating. After the curing process, the conveyor 120 carries the bottles to a further container processing stage, e.g., labelling, inspection, packing and/or filling.

A topcoating material as described herein will impart a desired color to a bottle, will increase abrasion and impact resistance of the glass container, will be waterproof and unaffected by the contents of any food or beverage, will be glossy and will not be abraded by like material, and will cover flaws and irregularities on the surface of glass containers such as to render them nearly invisible.

It has been demonstrated that the heat-curable color coating material can be cured quickly with hot convective air, easily achieved with commercial equipment. It is necessary to achieve a glass substrate temperature of 148.9°C (300°F) to achieve all of the desired properties of the color coat. Other curing processes are available.

It will be appreciated that further modifications could be made to the embodiment disclosed above while still obtaining many of these advantages and without departing from the scope of the invention as described in the appended claims.

## Claims

1. A method of coating a glass container, comprising the steps of: providing a container of glass, said glass having an inside surface directed toward an interior of said container and an outer surface directed toward an exterior of said container; annealing said glass container; coating said container with at least a final acrylic coating layer applied in liquid form; and curing said acrylic coating; said method being characterized by the steps of applying a first coating material to said container at a first location in a container fabrication line subsequent to said annealing step; conveying said container to a second location with said first coating material providing surface lubricity; and applying an acrylic coating layer which is compatible with said first coating material over said glass on said outer surface of said container while at least some of said first coating material remains on said outer surface, said acrylic coating layer having a cured thickness of no greater than 0.0152 mm (0.0006 inch).

2. A method according to claim 1, wherein said glass is substantially clear.

3. A method according to claim 1 or 2, wherein said acrylic coating layer is clear.

4. A method according to claim 1 or 2, wherein said acrylic coating layer is coloured.

5. A method according to any one of claims 1 to 4, wherein said coating layer is heat-curable.

6. A method according to claim 5, wherein said step of applying said acrylic coating includes the step of curing said coating in no more than 1.5 minutes by application of heat.

7. A method according to any one of claims 1 to 4, wherein said coating layer is UV-curable.

8. A method according to any foregoing claim, wherein said first coating material is ammonium stearate.

9. A method according to any foregoing claim, wherein the impact resistance of the initially provided glass container is increased by at least 30% on having said acrylic coating layer applied thereto.

10. A method according to any foregoing claim, wherein said coating layer contains a light blocking agent for blocking at least one predetermined wavelength of light in addition to any light blocked by any colour of said coating.

11. A method according to claim 10, wherein said predetermined wavelength is ultraviolet.

12. A method according to claim 10, wherein siad predetermined wavelength is outside of the ultraviolet region.

13. A method of coating a glass container, comprising the steps of: providing a container of glass, said glass having an inside surface directed toward an interior of said container and an outer surface directed toward an exterior of said container; annealing said glass container; coating said glass container with at least a final acrylic coating layer applied in liquid form; and curing said acrylic coating; said method being characterized by the steps of applying a first coating material to said container at a first location in a container fabrication line subsequent to said annealing step; conveying said container to a second location with said first coating material providing surface lubricity; exposing said first coating material to an oxidizing flame whereby first coating material is burnt off; and applying an acrylic coating layer over said glass on said outer surface of said container subsequent to said oxidizing flame step, said acrylic coating layer having a cured thickness of no greater than 0.0152 mm (0.0006 inch).

## Patentansprüche

1. Verfahren zum Beschichten eines Glasbehälters, das die folgenden Schritte aufweist:
- Bereitstellen eines Behälters aus Glas, wobei das Glas eine innere Oberfläche, die zu der Innenseite des Behälters gerichtet ist, und eine äußere Oberfläche hat, die zu der Außenseite des Behälters gerichtet ist;
- Tempern des Glasbehälters;
- Beschichten des Behälters mit wenigstens einer letzten Acrylüberzugsschicht, die in flüssiger Form aufgebracht wird; und
- Aushärten des Acrylüberzugs;
wobei das Verfahren durch die folgenden Schritte gekennzeichnet ist:
- Aufbringen eines ersten Überzugsmaterials auf den Behälter an einem ersten Ort in einer Behälterfertigungsstraße anschließend an den Temperschritt;
- Transportieren des Behälters zu einem zweiten Ort, wobei das erste Überzugsmaterial eine Oberflächenlubrizität bietet; und
- Aufbringen einer Acrylüberzugsschicht, die mit dem ersten Überzugsmaterial kompatibel ist, über dem Glas auf der äußeren Oberfläche des Behälters, während gleichzeitig wenigstens ein Teil des ersten Überzugsmaterials an der äußeren Oberfläche verbleibt, wobei die Acrylüberzugsschicht eine ausgehärtete Dicke von nicht mehr als 0,0152 mm (0,0006 inch) hat.

2. Verfahren nach Anspruch 1,
wobei das Glas im wesentlichen klar ist.

3. Verfahren nach Anspruch 1 oder 2,
wobei die Acrylüberzugsschicht klar ist.

4. Verfahren nach Anspruch 1 oder 2,
wobei die Acrylüberzugsschicht farbig ist.

5. Verfahren nach einem der Ansprüche 1 bis 4,
wobei die Überzugsschicht wärmehärtbar ist.

6. Verfahren nach Anspruch 5,
wobei der Schritt des Aufbringens des Acrylüberzugs den Schritt des Aushärtens des Überzugs in nicht mehr als 1,5 Minuten durch Aufbringen von Wärme aufweist.

7. Verfahren nach einem der Ansprüche 1 bis 4,
wobei die Überzugsschicht UV-härtbar ist.

8. Verfahren nach einem der vorhergehenden Ansprüche,
wobei das erste Überzugsmaterial Ammoniumstearat ist.

9. Verfahren nach einem der vorhergehenden Ansprüche,
wobei die Schlagfestigkeit des anfänglich bereitgestellten Glasbehälters nach dem Aufbringen der Acrylüberzugsschicht um wenigstens 30 % erhöht wird.

10. Verfahren nach einem der vorhergehenden Ansprüche,
wobei die Überzugsschicht ein Lichtblockiermittel enthält, um wenigstens eine vorbestimmte Lichtwellenlänge zusätzlich zu dem durch eine Farbe des Überzugs blockierten Licht zu blockieren.

11. Verfahren nach Anspruch 10,
wobei die vorbestimmte Wellenlänge Ultraviolett ist.

12. Verfahren nach Anspruch 10,
wobei die vorbestimmte Wellenlänge außerhalb des UV-Bereichs ist.

13. Verfahren zum Beschichten eines Glasbehälters, das die folgenden Schritte aufweist:
- Bereitstellen eines Behälters aus Glas, wobei das Glas eine innere Oberfläche, die zu der Innenseite des Behälters gerichtet ist, und eine äußere Oberfläche hat, die zu der Außenseite des Behälters gerichtet ist;
- Tempern des Glasbehälters;
- Beschichten des Glasbehälters mit wenigstens einer letzten Acrylüberzugsschicht, die in flüssiger Form aufgebracht wird; und
- Aushärten des Acrylüberzugs;
wobei das Verfahren durch die folgenden Schritte gekennzeichnet ist:
- Aufbringen eines ersten Überzugsmaterials auf den Behälter an einem ersten Ort in einer Behälterfertigungsstraße anschließend an den Temperschritt;
- Transportieren des Behälters zu einem zweiten Ort, wobei das erste Überzugsmaterial eine Oberflächenlubrizität bietet;
- Beaufschlagen des ersten Überzugsmaterials mit einer oxidierenden Flamme, so daß dadurch erstes Überzugsmaterial abgebrannt wird; und
- Aufbringen einer Acrylüberzugsschicht über dem Glas auf der äußeren Oberfläche des Behälters anschließend an den Schritt der Behandlung mit der oxidierenden Flamme, wobei die Acrylüberzugsschicht eine ausgehärtete Dicke von nicht mehr als 0,0152 mm (0,0006 inch) hat.

## Revendications

1. Procédé pour revêtir un récipient en verre comprenant les étapes de : fournir un récipient en verre, ledit verre ayant une surface intérieure dirigée en direction d'un intérieur dudit récipient et une surface extérieure dirigée vers l'extérieur dudit récipient ; recuire ledit récipient en verre ; revêtir ledit récipient avec au moins une couche de revêtement acrylique finale appliquée sous forme liquide ; et cuire ledit revêtement acrylique ; ledit procédé étant caractérisé par les étapes d'appliquer un premier matériau de revêtement audit récipient en un premier endroit dans la chaîne de fabrication de récipient après ladite étape de recuisson ; de convoyer ledit récipient vers un second endroit avec ledit premier matériau de revêtement fournissant une lubricité de surface ; et d'appliquer une couche de revêtement acrylique qui est compatible avec ledit premier matériau de revêtement sur ledit verre sur ladite surface externe dudit récipient pendant qu'au moins une partie dudit premier matériau de revêtement reste sur ladite surface externe, ladite couche de revêtement acrylique ayant une épaisseur cuite pas supérieure à 0,0152 mm (0,0006 pouce).

2. Procédé selon la revendication 1, dans lequel ledit verre est substantiellement transparent.

3. Procédé selon la revendication 1 ou 2, dans lequel ladite couche de revêtement acrylique est transparente.

4. Procédé selon la revendication 1 ou 2, dans lequel ladite couche de revêtement acrylique est colorée.

5. Procédé selon l'une quelconque des revendications 1 à 4, dans lequel ladite couche de revêtement peut être cuite à chaud.

6. Procédé selon la revendication 5, dans lequel ladite étape d'appliquer ledit revêtement acrylique comprend l'étape de cuire ledit revêtement en pas plus de 1,5 minute par application de chaleur.

7. Procédé selon l'une quelconque des revendications 1 4, dans lequel ladite couche de revêtement peut être cuite par rayons ultra-violet.

8. Procédé selon l'une quelconque des revendications précédentes, dans lequel ledit premier matériau de revêtement est du stearate d'ammonium.

9. Procédé selon l'une quelconque des revendications précédentes, dans lequel la résistance à l'impact du récipient en verre fournit initialement est augmentée d'au moins 30% en ayant ladite couche de revêtement acrylique appliquée dessus.

10. Procédé selon l'une quelconque des revendications précédentes, dans lequel ladite couche de revêtement contient en agent bloquant la lumière pour bloquer au moins une longueur d'onde prédéterminée de lumière en plus de toute lumière bloquée par toute couleur dudit revêtement.

11. Procédé selon la revendication 10, dans lequel ladite longueur d'onde prédéterminée est l'ultra-violet.

12. Procédé selon la revendication 10, dans lequel ladite longueur d'onde prédéterminée est à l'extérieur de la zone ultra-violet.

13. Procédé pour revêtir un récipient en verre, comprenant les étapes de : fournir un récipient en verre, ledit verre ayant une surface intérieure dirigée vers l'intérieur dudit récipient et une surface extérieure dirigée vers un extérieur dudit récipient ; recuire ledit récipient en verre ; revêtir ledit récipient en verre avec au moins une couche de revêtement acrylique finale appliquée sous forme liquide ; et cuire ledit revêtement acrylique ; ledit procédé étant caractérisé par les étapes d'appliquer un premier matériau de revêtement audit récipient en un premier endroit dans une chaîne de fabrication du récipient après ladite étape de recuisson ; de convoyer ledit récipient vers un second endroit avec ledit premier matériau de revêtement fournissant une lubricité de surface ; d'exposer ledit premier matériau de revêtement à une flamme oxydante de sorte que le premier matériau de revêtement est brûlé ; et d'appliquer une couche de revêtement acrylique sur ledit verre sur ladite surface extérieure dudit récipient après ladite étape de flamme oxydante ; ladite couche de revêtement acrylique ayant une épaisseur cuite de pas plus de 0,0152 mm (0,0006 pouce).
